

## UNITED STATES PATENT OFFICE

1,970,141

PROCESS FOR HARDENING IRON, STEEL,  
AND CAST IRON ALLOYS BY NITRIDINGOtto Hengstenberg, Essen, Germany, assignor, by  
mesne assignments, to The Nitralloy Corpora-  
tion, a corporation of DelawareNo Drawing. Application October 10, 1931,  
Serial No. 568,209. In Germany November 1,  
1930

4 Claims. (Cl. 148—16)

The invention relates to processes for hardening iron, steel, and cast iron, alloys by nitriding and has for its object to improve these processes in so far as a greater nitride depth is obtained 5 than it was hitherto possible, as well as an increased hardness of the nitrided layer.

It is known that heated metal surfaces such as those of the alloys of iron, steel and cast iron that are suitable for nitriding, act catalytically upon ammonia gases contacted therewith thereby accelerating the dissociation of the ammonia. Similarly, certain of the metals used in constructing containers for nitriding act catalytically upon ammonia at nitriding temperatures. At the same time, it has been found that better and more uniform nitriding results are obtained when the percentage dissociation of the ammonia gas passed over the surfaces intended to be nitrided is kept within certain limits, advantageously 15 within a range of about 30 to 40%. Owing to the catalytic effect of the heated metal surfaces exposed to the ammonia it has been heretofore difficult to control the percentage dissociation of the ammonia within the desired range except by increasing the rate of circulation of the ammonia through the nitriding container, and this method has proven relatively expensive because of the increased consumption of the ammonia. Furthermore, increase of the rate of circulation of 20 the ammonia does not entirely prevent a higher percentage dissociation of the ammonia in the localized areas where the ammonia gas contacts with the hot metal surfaces of the articles being nitrided.

It has been found that substances which act as catalyst poisons in the manufacture of ammonia also serve to bring about an increase in the hardness and depth of the hardness layer in nitride hardening. These substances serve to inhibit the catalytic action of the metal surfaces upon the ammonia gas and thereby retard the decomposition of the ammonia. In this way control of the rate of decomposition of the ammonia through control of the nitriding temperature and the rate 45 of the circulation of the ammonia is made certain.

The improved results above mentioned may be obtained by carrying out the nitriding in the presence of a metal oxide, such for example as cobalt oxide, which is decomposable under the conditions obtaining in the nitriding operation to yield 60 the catalyst poison. I have also used cobalt sulphate with similar results.

In carrying the invention into effect the articles to be hardened may, for example, be sprinkled with a thin layer of pulverized cobalt oxide and then nitrided in the usual way in a steam of ammonia at about 500° C., the cobalt oxide being reduced during the nitriding and the decomposition products acting as catalyst poisons. By this process with a given duration of the nitriding 70 treatment, a greater nitriding depth is produced than with a nitriding treatment of the same duration without the use of a catalyst poison.

What I claim and desire to secure by Letters Patent is:—

1. In the art of hardening ferrous base alloys by nitriding, the improvement which comprises treating such an alloy with ammonia gas at a nitriding temperature in the presence of a substance selected from the group consisting of 80 cobalt oxide and cobalt sulphate.

2. In the art of hardening ferrous base alloys by nitriding, the improvement which consists in nitriding such an alloy while contacting said alloy with a substance selected from the group 85 consisting of cobalt oxide and cobalt sulphate.

3. In the art of hardening ferrous base alloys by nitriding, the improvement which comprises treating such an alloy with ammonia gas at a nitriding temperature while contacting said alloy 90 with finely divided cobalt oxide.

4. In the art of hardening ferrous base alloys by nitriding, the improvement which comprises treating such an alloy with ammonia gas at a nitriding temperature while contacting said alloy 95 with finely divided cobalt sulphate.

OTTO HENGSTENBERG.

100